



US005334573A

# United States Patent [19]

## Schild

[11] Patent Number: 5,334,573  
[45] Date of Patent: Aug. 2, 1994

[54] **SHEET MATERIAL FOR THERMAL TRANSFER IMAGING**

[75] Inventor: **Howard G. Schild**, Brighton, Mass.

[73] Assignee: **Polaroid Corporation**, Cambridge, Mass.

[21] Appl. No.: **801,460**

[22] Filed: **Dec. 2, 1991**

[51] Int. Cl.<sup>5</sup> ..... **B41M 5/035; B41M 5/38**

[52] U.S. Cl. ..... **503/227; 428/195; 428/419; 428/480; 428/500; 428/913; 428/914**

[58] Field of Search ..... 8/471; 428/195, 913, 428/914, 419, 480, 500; 503/227

[56] **References Cited**

**U.S. PATENT DOCUMENTS**

4,555,427 11/1985 Kawasaki et al. ..... 428/195  
4,615,938 10/1986 Hotta et al. ..... 428/323  
4,626,256 12/1986 Kawasaki et al. ..... 8/471  
4,721,703 1/1988 Kabayashi et al. ..... 503/227  
4,820,687 4/1989 Kawasaki et al. ..... 503/227  
4,914,078 4/1990 Hann et al. ..... 503/227

4,997,807 3/1991 Mukoyoshi et al. ..... 503/227  
5,024,989 6/1991 Chiang et al. ..... 503/227

**FOREIGN PATENT DOCUMENTS**

407615A1 1/1991 European Pat. Off. ..... 503/227  
0223862 11/1985 Japan ..... 503/227  
0223878 11/1985 Japan ..... 503/227  
63-247397 6/1990 Japan ..... 503/227

**OTHER PUBLICATIONS**

Patent Abstracts of Japan, vol. 14, No. 351.

Primary Examiner—B. Hamilton Hess

Attorney, Agent, or Firm—Carol A. Loeschorn; Edward W. Black

[57] **ABSTRACT**

Sheet materials for use in thermal transfer imaging systems comprising a donor sheet and a receiving sheet are provided wherein the donor sheet and the receiving sheet do not stick to each other during thermal processing.

**36 Claims, No Drawings**

## SHEET MATERIAL FOR THERMAL TRANSFER IMAGING

### BACKGROUND OF THE INVENTION

#### 1. Field of the Invention

This invention relates to a sheet material for use in a thermal transfer imaging system comprising a receiving sheet and a donor sheet. More particularly, it relates to a thermal imaging system wherein the donor sheet and receiving sheet do not stick to each other during thermal processing.

#### 2. Description of the Related Art

Thermal transfer imaging processes wherein one or more thermally transferable dyes are transferred from a donor sheet to a receiving sheet in response to heat are well known. Such imaging processes employ imaging media consisting of a donor sheet comprising a dye or dyes and a binder for the dyes which is placed adjacent to a receiving sheet suitable for receiving the transferred dye(s). The imaging process comprises heating selected portions of the donor sheet in accordance with image information to effect an imagewise transfer of the dye(s) to the receiving sheet, thereby forming an image on the receiving sheet.

To enhance the image-receiving capability of the image-receiving sheet and thereby obtain higher density images, resins having a low glass transition point and softening point, e.g., polyester resins, are generally coated on the image-receiving sheet. However, when imaging is effected, heat is applied at high temperatures e.g., generally 200° C. or higher when a thermal print-head is employed. The high temperatures cause softening and/or melting of the resin in the image-receiving sheet and the binder for the dyes in the dye donor sheet resulting in adhesion between the two sheets. This adhesion results in sticking and subsequent tearing of the two sheets upon separation from each other.

To eliminate this thermal sticking, it has been suggested to incorporate a dye-permeable release agent in either the donor or receiving sheet which allows for dye transfer but prevents adhesion of the donor sheet to the receiving sheet during printing. The release agent can be employed either as a discrete layer on top of the receiving material or the dye layer in the donor sheet, or the release agent can be blended in with the receiving material before coating.

Materials previously employed as release agents include silicone-based oils, poly(organosiloxanes), fluorine-based polymers, fluorine- or phosphate-containing surfactants, fatty acid surfactants and waxes. The inherently different chemical structure of the release agents from that of the dyes to be transferred leads to an interfacial barrier at the donor/receiver interface causing decreased dye densities in the image-receiving sheet. These materials are surface-active which promotes their presence at the receiving sheet/donor sheet interface where they additionally contribute desired slip properties and frictional characteristics to the image-receiving surface to prevent sticking. However, these release agents tend to be migratory and can be rubbed off the surface by touch, providing areas where sticking can occur. They also attract dirt and dust which degrades image quality.

Crosslinking of various release materials has been proposed to hold the release material in place and to alleviate some of the above problems. U.S. Pat. No. 4,626,256 issued Dec. 2, 1986, U.S. Pat. No. 4,820,687

issued Apr. 11, 1989, and U.S. Pat. No. 4,914,078 issued Apr. 3, 1990 disclose image-receiving layers containing dye-permeable releasing agents comprising hardened type (crosslinked) silicone oils. However, there are disadvantages to having a separate crosslinked material. Not only is there a decrease in dye density due to the inherently different chemical structure of the silicone oils from that of the dyes, but crosslinking additionally causes a decrease in the transferred dye density. The temperature requirements of thermally induced crosslinking processes limit the types of support materials that may be utilized for the receiving sheet. Moreover, certain release materials, most notably the silicone oils and crosslinked silicone oils, make it difficult to laminate the image-receiving sheet to other materials because they inhibit the laminating adhesive from adhering to the image-receiving sheet. Further, the release materials make it difficult to write on the image-receiving sheet because they interfere with ink adhesion at the image-receiving surface.

It has also been suggested to increase the heat resistance of the image-receiving material to prevent softening of the receiving material and hence alleviate sticking. U.S. Pat. No. 4,721,703, issued Jan. 26, 1988, discloses a receiving sheet comprising a base material and a coating composition, the coating composition consisting essentially of a thermoplastic resin for receiving a dye and a compound having two or more free radical polymerizable ethylenically unsaturated double bonds in one molecule, the coating being crosslinked. The resulting receiving sheet is described as being substantially non-heat bondable (does not stick) to the dye layer by virtue of the heat resistance imparted by the crosslinked polymer therein. However, this method is disadvantageous in that crosslinked materials generally result in decreased dye densities and require an additional processing step.

U.S. Pat. No. 4,997,807, issued Mar. 5, 1991, discloses a receiving sheet which is described as free from blocking (sticking of the receiving sheet to the donor sheet during thermal processing). The receiving sheet comprises a support having thereon an image-receiving layer formed by coating a substantially solvent-free coating composition comprising (A) a macromonomer dyeable with a sublimable dye and containing a radical polymerizable functional group at one terminal of the molecular chain thereof, said macromonomer being solid at room temperature, dissolved in (B) a liquid radiation-curable monomer and/or oligomer on a support and irradiating the coat with radiation. According to the examples given in the patent, excellent blocking results were obtained only when a polyfunctional monomer and a siloxane were present. This suggests that both crosslinking and a surface active agent (release agent) are necessary in order to obtain the best results.

U.S. Pat. No. 4,555,427, issued Nov. 26, 1985, discloses a heat transferable sheet (receiving sheet) comprising a receptive layer which receives a dye transferred from a heat transfer printing sheet upon being heated, the receptive layer comprising first and second regions having the following properties:

(a) The first region is formed from a synthetic resin having a glass transition temperature of from -100° to 20° C., preferably from -50° to 10° C., and having polar groups such as an ester linkage, C—CN linkage and C—C1 linkage.

(b) The second region is formed from a synthetic region having a glass transition temperature of at least 40° C., preferably from 50° to 150° C., and preferably the second region-forming synthetic resin has also a polar group.

(c) Both the first region and the second region are exposed at the surface of the receptive layer, and the first region occupies at least 15%, preferably from 15 to 95% of the surface.

(d) The first region is present in the form of mutually independent islands, the respective longitudinal length of which is from 0.5 to 200  $\mu\text{m}$ , preferably from 10 to 100  $\mu\text{m}$ , and desirably the periphery of the first region is substantially surrounded by the second region.

According to the examples given in the patent, hardened silicone oils were added to enhance the releasability of the heat transfer printing sheet upon being heated.

#### SUMMARY OF THE INVENTION

The present invention provides a sheet material for use in thermal transfer imaging systems which avoids sticking, i.e., the thermal fusing of the donor sheet and the image-receiving sheet during thermal processing, by employing an image-receiving polymer system which is incompatible/immiscible with the donor polymer system. Since the two polymer systems are incompatible/immiscible at the temperature and time which they are in contact, i.e., during thermal processing, there is no thermal adhesion between the donor sheet and the image-receiving sheet.

Specifically, the present invention provides thermal transfer imaging systems comprising a donor sheet and a receiving sheet, the donor sheet comprising a support, an image-forming material capable of being transferred by heat and a polymer system comprising at least one polymer as a binder for the image-forming material, and the receiving sheet comprising a polymer system comprising at least one polymer capable of receiving said image-forming material from said donor sheet upon application of heat thereto, the polymer system of said receiving sheet being incompatible/immiscible with the polymer system of said donor sheet at the receiving sheet/donor sheet interface so that there is no adhesion between the donor sheet and the receiving sheet during thermal processing, said polymer system of the donor sheet and said polymer system of the receiving sheet being substantially free of a release agent, such as silicone-based oils, poly(organosiloxanes), fluorine-based polymers, fluorine- or phosphate-containing surfactants, fatty acid surfactants and waxes.

The present invention further provides for a method of thermal transfer imaging employing the above described sheet materials.

By avoiding the use of a separate release agent, the present invention provides images of higher dye densities. Since no post-coating crosslinking is necessary, a one-step process produces the image-receiving sheet and dye densities are not compromised. Since no heat, other than moderate drying temperatures is required, thermal distortion of the support material is avoided. Moreover, since the present invention lacks a silicone oil or other low surface energy release agent, lamination of the image-receiving sheet to other materials is easier as is writing with ink on the surface of the image.

#### DETAILED DESCRIPTION OF THE INVENTION

As noted above, the sheet materials of the present invention are used in thermal transfer imaging systems. The donor sheet comprises a support and an image-forming material capable of being transferred by heat and at least one polymer as a binder for the image-forming material. The image-forming material can be a dye or other image-forming material which transfers by diffusion or sublimation, upon application of heat, to the image receiving sheet to form an image therein. It will be understood that where multicolor images are desired, the donor sheet would comprise additional dyes or other image-forming materials. The image-receiving sheet comprises a polymer system comprising at least one polymer capable of receiving said image-forming material from said donor upon the application of heat thereto, the polymer system of said receiving sheet being incompatible/immiscible with the polymer system of the donor sheet at the receiving sheet/donor sheet interface so as to inhibit thermal adhesion between the donor and receiving sheets during thermal processing. The polymer system employed as binder for the image-forming material and the polymer system of the receiving sheet are substantially free of release agents, such as silicone-based oils, poly(organosiloxanes), fluorine-based polymers, fluorine- or phosphate-containing surfactants, fatty acid surfactants and waxes. "Substantially free of" means that none of these materials are intentionally added to aid release. Selected portions of the donor sheet are heated in accordance with image information so as to transfer dye or other image-forming material from the donor sheet to the receiving sheet to form an image thereon.

The image-receiving polymer system of the present invention may be coated on a support or it may be self-supporting.

The terms incompatible and immiscible are used interchangeably but the latter is the preferred term according to *The Encyclopedia of Polymer Science and Engineering*, John Wiley & Sons, 1988, vol. 12, p. 399.

By definition, two polymers are considered to be immiscible if when they are "in contact" (the geometry of which is very much a function of the method of preparation, e.g., melt-mixing, solution mixing, laminating, etc.) there is no intimate mixing, i.e., there are gross symptoms of macroscopic phase segregation/separation into more than one phase.

In the present invention, the donor and receiving polymer systems are "in contact" during imaging and are immiscible at the temperature and time of contact, the latter being on the order of milliseconds, so that there is no mixing of the two and, therefore, no thermal adhesion of the donor and receiving sheets. Thus, while the image-receiving polymer(s) and the binders in the donor sheet may be softened by the temperatures of thermal processing, they are immiscible and, therefore, they do not adhere to each other.

The donor binder serves to keep the image-forming material dispersed uniformly and to prevent transfer or bleeding of the relatively low molecular weight image-forming material except where the donor sheet is heated during the thermal imaging. A necessary requirement, therefore, is that the binder be able to dissolve and/or disperse the dye. This necessarily excludes silicone-based oils, poly(organosiloxanes), fluorine-based polymers, fluorine- or phosphate-containing surfactants,

fatty acid surfactants and waxes since these materials, based on their inherent elemental structure, are not capable of keeping the dye uniformly dispersed. Suitable binders for the image-forming material, provided they are immiscible with the polymer system of the receiving sheet, include cellulose resins, such as, ethylcellulose, hydroxyethylcellulose, ethylhydroxyethylcellulose, hydroxypropylcellulose, cellulose acetate, and cellulose acetate butyrate; vinyl resins, such as, polyvinyl alcohol, polyvinyl pyrrolidone, polyvinyl acetate, vinyl alcohol/vinyl butyral copolymers; polyacrylamide resins, and acrylic acid resins, such as, poly(methyl methacrylate).

Desirably the weight ratio of dye or other image-forming material to binder is in the range of from about 0.3:1 to about 2.55:1, preferably about 0.55:1 to about 1.5:1.

The polymer system of the image-receiving sheet serves to enhance the receipt of dye or other image-forming material in the receiving sheet. Suitable polymer(s) which can be used as the image-receiving material must be able to receive dye (or other image-forming material) in order to maximize dye transfer. The polymer(s) used as the image-receiving material can also serve to provide mechanical strength to the receiving sheet and the finished image produced therefrom. Examples of such materials are extruded polymer films wherein the particular polymer chosen is both capable of receiving the image-forming material and providing the necessary mechanical strength.

Polymers which can be used as the image-receiving material include any of those commonly employed in the art as receiving materials provided they are immiscible with the polymer system of the donor sheet. For example, a polyester, polyacrylate, polycarbonate, poly(4-vinylpyridine), polyvinyl acetate, polystyrene and its copolymers, polyurethane, polyamide, polyvinyl chloride, polyacrylonitrile or a polymeric liquid crystal resin may be used as the image-receiving component. Desirably, the polymer for the image-receiving sheet is a polyester resin, preferably a polyester resin comprising aromatic diacids and aliphatic diols e.g., Vylon ® 103, Vylon ® 200, and Vylon ® MD-1200 (an aqueous polyester), all commercially available from Toyobo Co., Ltd., Tokyo, Japan and Vitel ® 2200 and Vitel ® 2700 commercially available from Goodyear Tire and Rubber Co., Polyester Division, Apple Grove, W.V. Silicone-based oils, poly(organosiloxanes), fluorine-based polymers, fluorine- or phosphate-containing surfactants, fatty acid surfactants and waxes are not suitable compounds to be used as image-receiving materials since they are not very good at receiving and holding onto dyes.

The thickness of the image-receiving layer will generally be in the range of about 0.5 to 5 microns ( $\mu$ ).

As noted above, the donor binder and receiving polymer(s) must be chosen such that they are immiscible with each other, upon contact and softening at the temperature and time of processing, so that no thermal adhesion of the two sheets will occur during processing. A single polymer as binder for the donor and a single polymer as the image-receiving material for the receiving sheet would be preferable; however, it may be necessary to use polymer blends in the donor and/or receiving sheet in order to optimize performance for a given system. The polymer blend chosen for either the donor or receiving sheet may be a homogeneous or heterogeneous blend.

In determining whether two polymers are immiscible one can look to the relevant art, wherein many studies of polymer-polymer compatibility/miscibility have been reported, to find pairs of polymers reported as immiscible. Alternatively, one may employ one of the several techniques which exist in the art to measure polymer-polymer miscibility. For a review of these various techniques see *The Encyclopedia of Polymer Science and Engineering*, John Wiley & Sons, 1985, vol. 3, pp. 760-765. However, these techniques result in measures of miscibility which are relative rather than absolute and depend upon the method of preparation of the polymer blend. Thus, where a polymer blend is found to be immiscible using one technique, another may indicate miscibility. For example, the degree of transparency of the polymer blend is employed as a measure of immiscibility. If the blend is transparent, it generally indicates the polymers are miscible; if translucent or opaque, it generally implies multiple phases and therefore, immiscibility. However, if the refractive indices of the two polymers are close or equal to each other or if the domains in a multiphase blend are smaller than the wavelength of light, the polymer blend may appear transparent even if the two polymers are immiscible.

In addition, miscibility between two polymers is affected by the presence of other substances and, therefore, the dye or other image-forming material in the donor sheet affects the interactions of the donor binder with the receiving-polymer and can influence miscibility. Additionally, the method of coating or choice of solvent from which to coat the polymer blend can impact miscibility. Thus, while determining immiscibility of the donor binder and receiving polymer by one of the available techniques or by locating a pair of polymers found to be immiscible in the literature does not insure that they will work for purposes of the present invention, it is a good starting point. Routine testing under the conditions of the present invention will readily determine if a preliminary finding of immiscibility is maintained under processing conditions.

When a support is employed in the image-receiving sheet, it serves to provide mechanical strength to the receiving sheet and the finished image. The support is not particularly limited, although preferably it should have a thickness of at least 100 microns ( $\mu$ ) and desirably 125 to 225  $\mu$ . If the support is of a thickness less than 100  $\mu$ , it is susceptible to thermal deformation during printing. The support may be a sheet or film and may be transparent or reflective. Examples of transparent supports include polyesters, polycarbonates, polystyrenes, cellulose esters, polyolefins, polysulfones, polyimides and polyethylene terephthalate. Reflective supports useful for the image-receiving sheet include cellulose paper, polyester coated cellulose paper, polymer coated cellulose paper, e.g., polyethylene or polypropylene coated paper, coated or uncoated wood-free paper, synthetic paper, and plastic films which carry a layer of reflective pigment or which include a filler, e.g., polyethylene terephthalate containing calcium carbonate or titanium dioxide. Also useful is a polyester film made opaque by the presence of voids, commercially available under the tradename "Melinex" from Imperial Chemical Industries (ICI) Films, England.

To avoid peeling or other damage to the image-receiving layer and/or the finished image due to poor adhesion of the image-receiving material to the support, a subcoat may be added to the face of the support which carries the image-receiving material to enhance adhe-

sion. For example, an anionic aliphatic polyester urethane polymer, applied as a subcoat, has been found to enhance adhesion to polyethylene cladded support materials.

The donor sheets used in the present invention can be those conventionally used in thermal dye diffusion transfer imaging systems. In systems of this type the image-forming material in the donor sheet is a dye. The dyes that can be used in the present process can be any of those used in prior art thermal diffusion or sublimation transfer processes. Typically, such a dye is a heat-sUBLIMABLE dye having a molecular weight of the order of about 150 to 800, preferably 350 to 700. In choosing a specific dye for a particular application, it may be necessary to take account of factors such as heat sublimation temperature, chromaticity, compatibility with any binder used in the donor sheet and compatibility with any image receiving materials on the receiving sheet. Specific dyes previously found to be useful include:

Color Index (C.I.) Yellows Nos. 3, 7, 23, 51, 54, 60 and 79;

C.I. Disperse Blues Nos. 14, 19, 24, 26, 56, 72, 87, 154, 165, 287, 301, and 334;

C.I. Disperse Reds Nos. 1, 59, 60, 73, 135, 146 and 167;

C.I. Disperse Violets Nos. 4, 13, 31, 36 and 56;

C.I. Solvent Violet No. 13;

C.I. Solvent Black No. 3;

C.I. Solvent Green No. 3;

C.I. Solvent Yellows Nos. 14, 16, 29 and 56;

C.I. Solvent Blues Nos. 11, 35, 36, 49, 50 63, 97, 70, 105 and 111; and

C.I. Solvent Reds Nos. 18, 19, 23, 24, 25, 81, 135, 143, 146 and 182.

One specific set of dyes which have been found to give good results in a three-color thermal imaging process of the present invention are:

Yellow C.I. Disperse Yellow No. 231, also known as Foron Brilliant Yellow S-6GL;

Cyan C.I. Solvent Blue No. 63, C.I. No. 61520, 1-(3, -methylphenyl)amino-4-methylaminoanthraquinone;

Magenta A [mixture of approximately equal amounts of C.I. Disperse Red No. 60, C.I. No. 60756, 1-amino-2-phenoxy-4-hydroxyanthraquinone, and C.I. Disperse 45 Violet No. 26, C.I. No. 62025, 1,4-diamino-2,3-diphenoxanthraquinone].

The donor sheets of the present invention may also be those used in thermal transfer systems which utilize in situ dye generation to form images. In systems of this type, the image-forming material in the donor sheet is a material which, upon application of heat, transfers to the receiving sheet. The transferred image-forming component combines with a material already present in the receiving sheet to generate the desired color. Such systems are described, e.g., in U.S. Pat. No. 4,824,822 and U.S. Pat. No. 5,011,811.

The donor sheet used in the present process conveniently comprises a layer of image-forming material disposed on one face of the support, the layer comprising the image-forming material and a binder for the image-forming material. During thermal imaging, the layer of image-forming material on the support faces the receiving sheet. The support may be paper, for example condenser paper, or a plastic film, for example an aromatic polyamide film, a polyester film, a polystyrene film, a polysulfone film, a polyimide film or a polyvinyl film. The thickness of the support is usually in the range

of about 2  $\mu$  to about 10  $\mu$ , although it is desirable to keep the thickness of the support in the range of about 4 to about 7  $\mu$ , since a thick support delays heat transfer from the printing head to the dye and may affect the resolution of the image produced. A donor sheet having a 6  $\mu$  polyethylene terephthalate support has been found to give good results in the present process.

Desirably, a layer of a lubricating agent is present on the back of the donor sheet remote from the dye layer, 10 the lubricating agent serving to reduce adhesion of a thermal printing head to the donor sheet. Such a layer of lubricating agent (also called "heat-resistant slipping layers"), and methods for its creation on a donor sheet are described in detail in U.S. Pat. No. 4,720,480, issued 15 Jan. 19, 1988, and hence such lubricating agents will not be described in detail herein. A preferred lubricating agent comprises (a) a reaction product between polyvinyl butyral and an isocyanate; (b) an alkali metal salt or an alkaline earth metal salt of a phosphoric acid ester; 20 and (c) a filler. This lubricating agent may also comprise a phosphoric acid ester free of salts.

The filler used in this preferred lubricating agent can be an inorganic or organic filler having heat resistance, for example, clay, talc, a zeolite, an aluminosilicate, 25 calcium carbonate, polytetrafluoroethylene powder, zinc oxide, titanium oxide, magnesium oxide, silica and carbon. Good results have been achieved in the present process using a lubricating layer containing as filler talc particles with an average size of 1 to 5  $\mu$ .

30 Because it is desirable to keep the donor sheet thin, for reasons already discussed above, the thickness of the lubricating layer preferably does not exceed about 5  $\mu$ .

The heat required for thermal transfer may be provided by a thermal printhead or by any other suitable 35 means, e.g., by irradiation with a laser beam as known in the art.

The present invention is described in more detail by the following examples.

The sheet materials of each example were thermally 40 processed using a Hitachi VY-200 thermal printer, sold by Hitachi Ltd., Tokyo, Japan, to print a multi-color test pattern.

All optical reflection densities were measured using an X-Rite 338 photographic densitometer.

#### EXAMPLE 1

This Example illustrates the preparation of a sheet material according to the present invention and its use in thermal imaging. The donor sheet comprised a support layer of polyethylene terephthalate carrying a dye layer comprised of dye dispersed in poly(methyl methacrylate) (PMMA). The donor sheet was in the form of a long roll comprising a plurality of panes, each pane containing a single color dye or dye mixture, with yellow, cyan and magenta panes being repeated cyclically along the film so that each triplet of three panes contained one pane of each color. One triplet of three panes is used for each print. The yellow pane comprised two pyridone dyes. The cyan pane comprised two anthraquinone dyes, and the magenta pane comprised three anthraquinone dyes.

The literature, e.g., Journal of Applied Polymer Science, 41 (11-12) pp. 2691-2704 (1990), has reported that poly(caprolactone) (PCL) is incompatible with PMMA, and therefore, a receiving sheet was prepared with PCL as the dye receiving material. A 10% w/v solution of PCL in chloroform was coated with a Meyer rod (#20) 65 onto a 4 rail (100  $\mu$  thick) 6"  $\times$  6" (15  $\times$  15 cm) opaque

polyester terephthalate support containing voids containing titanium dioxide (commercially available under the trade name Melinex ® 329, from Imperial Chemical Industries (ICI) Films, England), and dried in a ventilation hood at room temperature. The thickness of PCL was approximately  $2\mu$ . The coated sheet was cut to size, and the sheet was thermally printed. There was no sticking of the donor and receiving sheets. The measured dye densities are reported in Table I.

TABLE 1

|           | DYE DENSITIES |      |         |        |
|-----------|---------------|------|---------|--------|
|           | Black         | Cyan | Magenta | Yellow |
| Example 1 | 1.00          | 0.95 | 0.78    | 0.43   |

The foregoing data demonstrates that PCL and PMMA maintain their immiscibility under the thermal processing conditions of Example 1 and thus prevent sticking of the donor and receiving sheet during thermal processing. The data in Table 1 show that PCL receives 20

### EXAMPLE 2

A receiving sheet was prepared and processed as in Example 1, except that the polyester resin, Vylon ® 200, replaced the PCL. This system exhibited essentially total sticking of the donor and receiving sheets during thermal processing indicating the combination of PMMA and Vylon ® 200 for the donor and receiving sheet materials were not immiscible.

### EXAMPLE 3

PCL was blended with Vylon ® 200, the polyester resin of Example 2. Five-sheet materials were prepared and processed according to Example 1 except that the image-receiving sheets were prepared as follows: varying ratios of a solution of 16.8% (w/v) Vylon ® 200 in methyl ethyl ketone (MEK) and a 10% (w/v) solution of PCL in chloroform were mixed and coated onto a 4 mil Melinex ® 329 support with a #20 Meyer Rod and dried at room temperature in a ventilation hood to yield a thickness of approximately  $2\mu$ . The percentage (w/w) of PCL in each receiving sheet is reported in Table 2 as are the measured reflectance densities for the cyan, magenta and yellow regions and the visible reflection density for the black region of the test pattern. With 9.3% (w/w) PCL in the receiving material, there was significant sticking and consequently the dye densities could not be measured; however, at all other percentages of PCL reported in Table 2, no sticking was observed. To provide a control, the experiment was repeated using an experimental receiving sheet comprising a Melinex ® 329 support and a dye receiving layer comprising a polyester resin for receiving the dye and a thermally cured silicone release material comprising an epoxy-modified silicone oil and amino-modified silicone oil. The reflectance densities for the control are shown in Table 2. There was no sticking observed for the control.

From the data it can be seen that at 9.3 (w/w) % PCL, there is significant sticking indicating that under those particular conditions, immiscibility between the donor sheet and receiving polymer system is not maintained. However, at higher concentrations of PCL, e.g., sticking was avoided. Further, at PCL concentrations of about 11%, processing led to significantly higher dye densities as compared with the control which utilized a crosslinked silicone release material to prevent sticking.

The data also demonstrate how polymer blends can be utilized in the receiving sheet to improve performance for a given system, i.e., absence of sticking and high transferred dye densities.

TABLE 2

|           | DYE DENSITIES        |                      |                      |                      |
|-----------|----------------------|----------------------|----------------------|----------------------|
|           | Black                | Cyan                 | Magenta              | Yellow               |
| 9.3% PCL  | Significant Sticking | Significant Sticking | Significant Sticking | Significant Sticking |
| 11.1% PCL | 2.51                 | 2.05                 | 2.51                 | 2.12                 |
| 11.5% PCL | 2.41                 | 1.95                 | 2.37                 | 2.04                 |
| 12.4% PCL | 2.08                 | 1.68                 | 2.15                 | 1.60                 |
| 14.4% PCL | 2.12                 | 1.70                 | 2.21                 | 1.58                 |
| Control   | 2.36                 | 1.69                 | 2.10                 | 1.53                 |

### EXAMPLE 4

This Example illustrates two additional sheet materials according to the present invention.

Based on their structural similarity to poly(caprolactone), two additional aliphatic polyesters, poly(2,2-dimethyl-1,3-propylene succinate) (PDPS) and poly(ethylene adipate) (PEA), were tested for their immiscibility with PMMA, the binder for the donor sheet, in a sheet material according to the present invention.

Two receiving sheets were prepared as in Example 3, except that the receiving material for one was a mixture of PDPS and Vylon ® 200 containing 9.6 wt. % PDPS, and the receiving material for the other employed a mixture of PEA and Vylon ® 200 (16.3 w/w % PEA). The donor sheet was the donor sheet described in Example 1, which uses PMMA as the binder for the dyes. There was no sticking of the donor and receiving sheets with either receiving sheet upon thermal processing. The measured reflectance densities are reported in Table 3.

From the foregoing data, it will be seen that the sheet material prepared according to the present invention did not result in sticking of the donor and receiving sheets during processing and produced images having good reflectance densities.

TABLE 3

|                  | DYE DENSITIES |      |         |        |
|------------------|---------------|------|---------|--------|
|                  | Black         | Cyan | Magenta | Yellow |
| 9.6 wt. %        | 2.44          | 2.10 | 2.56    | 2.25   |
| PDPS/Vylon ® 200 |               |      |         |        |
| 16.3 wt. %       | 2.44          | 2.02 | 2.50    | 2.26   |
| PEA/Vylon ® 200  |               |      |         |        |

### EXAMPLE 5

This Example illustrates the preparation of sheet materials according to the present invention and the use of these sheet materials in thermal imaging. This Example also repeats the experiments using a control which contains a crosslinked silicone release material to prevent sticking.

Two different receiving materials according to the present invention were prepared and coated onto various support materials to yield coated coverages approximately  $2\mu$  in thickness in accordance with Example 1. The two receiving materials were 1) a 10% (w/v) mixture of Vylon ® 200/PEA, (83.6/16.4 w/w %) in MEK and 2) a mixture of Vylon ® 200/PCL (83/17, w/w %) in MEK:methylene chloride ( $\text{CH}_2\text{Cl}_2$ ), prepared by combining 7.7 g of a 10% (w/v) solution of PCL/ $\text{CH}_2\text{Cl}_2$  with 37.7 g of a 10% (w/v) solution of

Vylon® 200/MEK. These receiving materials were each coated (using a #20 Meyer rod) onto separate 4 mil Melinex® 329 supports, 2 mil Toyobo K 1553 synthetic paper (made of polyethylene terephthalate compounded with fillers) available from Toyobo Co., Ltd., Tokyo, Japan, and in the case of Vylon® 200/PEA on an experimental paper comprising pigmented polyethylene terephthalate on a cellulose core. The coated receiving sheets were dried at room temperature. These image-receiving sheets were used in conjunction with the donor sheet of Example 1 and processed. There was no sticking of the donor and receiving sheets for any of the sheet materials during thermal processing. The reflectance densities are shown in Table 4. To provide a control, the experiment was repeated with a different receiving sheet. The receiving material for the control contained a mixture of Vylon® 200 and a release material comprising 2.5 w/w % of epoxy modified/amino modified silicone oils. This mixture was combined with a 50/50 v/v solution of MEK/toluene to yield a 10% solids solution and was coated with a #20 Meyer rod to yield a thickness of approximately 2  $\mu$  onto the above 3 supports, Melinex® 329, Toyobo and the experimental paper. The resulting sheets were heated for 5 minutes at 110° C. to cure the release material. The receiving sheet employing the Toyobo K 1553 support warped during the thermal curing, but it could still be processed; however, the experimental paper support became so distorted during the curing, it could not be put through the printer. The measured reflection densities for the controls are also shown in Table 4.

TABLE 4

|                               | DYE DENSITIES |      |         |        |
|-------------------------------|---------------|------|---------|--------|
|                               | Black         | Cyan | Magenta | Yellow |
| <b>Vylon®/PEA:</b>            |               |      |         |        |
| (Melinex®)                    | 2.29          | 1.70 | 2.32    | 2.09   |
| (Toyobo)                      | 2.06          | 1.60 | 2.21    | 1.85   |
| (Experimental Paper Support)  | 2.64          | 1.77 | 2.73    | 2.46   |
| <b>Vylon®/PCL:</b>            |               |      |         |        |
| (Melinex®)                    | 2.43          | 1.69 | 2.50    | 2.21   |
| (Toyobo)                      | 2.10          | 1.60 | 2.33    | 1.98   |
| <b>Control:</b>               |               |      |         |        |
| (Melinex®)                    | 2.06          | 1.57 | 2.26    | 1.55   |
| (Toyobo)                      | 1.88          | 1.54 | 2.17    | 1.64   |
| (Experimental Paper Support*) | —             | —    | —       | —      |

\*Could not be thermally printed due to warping.

From the foregoing data it can be seen that the process of the present invention produced images having significantly increased reflection density as compared with the control. The experimental data of Example 5 also demonstrate that the support materials which can be used according to the present invention are not as limited as those which can be used where thermal cross-linking of a release material is employed to prevent sticking. The sheet material of the present invention can be dried at low temperatures, room temperature when organic solvents are used, thereby avoiding the warping which can occur to heat-sensitive supports during thermal curing.

## EXAMPLE 6

This example illustrates the preparation of a sheet material according to the present invention and its use in thermal imaging.

The donor sheet is a commercially available material sold by Hitachi, Ltd., Tokyo, Japan designated Hitachi Cassette Color Video Printer Paper Ink Set, VY-SX100 A, high density 100 Series.

5 The donor sheet is believed to comprise a support layer of polyethylene terephthalate 10  $\mu$  in thickness. The support layer carries a dye layer which is 4  $\mu$  to 5  $\mu$  in thickness and comprises dye dispersed in a vinyl alcohol/vinyl butyral copolymer, which softens at 85° C. and serves as a binder for the dye.

10 The donor sheet is supplied commercially in a cartridge comprising a feed or supply spool and a take-up spool, the two spools having parallel axes and each being disposed within a substantially light-proof, cylindrical, synthetic resin housing. The opposed ends of the two cylindrical housings are interconnected by a pair of parallel rails, leaving between the two housings an open rectangular frame in which a single pane of the donor sheet can be exposed.

15 In the commercial cartridge, the donor sheet is in the form of a long roll comprising a plurality of panes, each pane containing a single color dye, with yellow, cyan and magenta panes being repeated cyclically along the film so that each triplet of three panes contains one pane of each color. One triplet of three panes is used for each print. The dyes used are believed to be as follows:

20 Yellow C.I. Disperse Yellow No. 231, also known as Foron Brilliant Yellow S-6GL;

25 Cyan C.I. Solvent Blue No. 63, C.I. No. 61520, 1-(3'-methylphenyl)amino-4-methylaminoanthraquinone;

30 Magenta A [mixture of approximately equal amounts of C.I. Disperse Red No. 60, C.I. No. 60756, 1-amino-2-phenoxo-4-hydroxyanthraquinone, and C.I. Disperse Violet No. 26, C.I. No. 62025, 1,4-diamino-2,3-diphenoxoanthraquinone].

35 The literature, e.g., A. Dondos and E. Pierri, Polymer Bulletin (Berlin) 16(6), pp. 567-569 (1986), has reported the incompatibility of polyvinyl acetate and polystyrene (PS). Based on the similarity in structure between polyvinyl acetate and vinyl alcohol/vinyl butyral copolymer, i.e., both are aliphatic polymers containing polar groups, PS was used as the image-receiving polymer for the receiving sheet.

40 Thus, a receiving sheet was prepared according to Example 1, except that PS replaced the PCL. The donor and receiving sheet were processed according to Example 1. There was no sticking of the donor and receiving sheets during processing. The measured reflectance densities are reported in Table 5.

TABLE 5

|           | DYE DENSITIES |      |         |        |
|-----------|---------------|------|---------|--------|
|           | Black         | Cyan | Magenta | Yellow |
| Example 6 | 0.87          | 1.14 | 1.03    | 0.45   |

50 The foregoing data show that the vinyl alcohol/vinyl butyral copolymer and polystyrene maintain their incompatibility under the conditions of the present Example and that polystyrene receives dye.

55 It should be noted that Vylon® 200 used in Example 2 results in severe sticking when used by itself as the receiving material with the donor of this example.

## Example 7

60 Liquid crystal polymers (LCP) have been disclosed as useful materials for receiving dyes and result in good dye densities, see U.S. Pat. No. 5,024,989, issued Jun. 18,

1991 to the same assignee as the present invention. However, LCPs have been found to cause undesirable sticking when used in conjunction with the donor sheet of Example 6. To prevent sticking and also achieve good dye densities, a receiving sheet was prepared using a blend of polystyrene and a LCP of the formula

1. Sheet materials for use in combination in thermal diffusion transfer imaging comprising a donor sheet and a receiving sheet, the donor sheet comprising a support, an image-forming material capable of being transferred by heat and a polymer system comprising at least one polymer as a binder for the image-forming material, and the receiving sheet comprising a polymer system com-



prepared according to the procedure described in the aforementioned U.S. Pat. No. 5,024,989. A 5% w/v solution of LCP in chloroform was combined with a 5% solution of PS in MEK to give a mixture containing 7.75% (w/w) PS/LCP. The resulting mixture was coated with a #20 Meyer Rod to yield a thickness of receiving material  $\sim 2 \mu$  after drying. This receiving sheet and the donor sheet as described in Example 6 were thermally imaged. No sticking occurred during processing. The measured reflectance densities are reported in Table 6. To provide a control, the experiment was repeated using the commercial donor sheet described in Example 6 and a commercial receiving sheet, also sold by Hitachi, Ltd., as part of the set for use with the commercial donor. The receiving sheet is separately designated Hitachi Video Print Paper VY-S.

The commercial receiving sheet is believed to comprise a support layer formed of polyethylene terephthalate film 150  $\mu$  in thickness and containing pigment particles, which act as an opacifying agent and render the base layer white in color, so that the images produced on the receiving sheet are seen against a white background. One face of the support layer carries a subcoat which is 8 to 10  $\mu$  in thickness and, superimposed over this subcoat, an image receiving layer, which is 1.5 to 2  $\mu$  in thickness and composed of a polyester resin. Additionally it is believed that the receiving sheet contains a release agent comprised of a crosslinked siloxane material. The subcoat serves to increase the adhesion of the image receiving layer to the underlying support layer. There was no sticking of the donor and receiving sheets during processing. The measured reflectance densities are shown in Table 6.

TABLE 6

|           | DYE DENSITIES |      |         |        |
|-----------|---------------|------|---------|--------|
|           | Black         | Cyan | Magenta | Yellow |
| Example 7 | 1.92          | 1.83 | 2.08    | 1.37   |
| Control   | 1.72          | 1.70 | 1.96    | 1.20   |

The foregoing data, particularly the data in Table 6, show that the process of the present invention produced images having significantly increased reflectance density relative to the control.

Since certain changes may be made in the herein described subject matter without departing from the scope of the invention herein involved, it is intended that all matter contained in the above description and Examples be interpreted as illustrative and not in a limiting sense.

I claim:

20 prising at least one polymer capable of receiving said image-forming material from said donor sheet upon application of heat thereto, the polymer system of said receiving sheet being incompatible/immiscible with the polymer system of said donor sheet at the receiving sheet/donor sheet interface so that there is no adhesion between the donor sheet and the receiving sheet during thermal processing, said donor sheet polymer system and said receiving sheet polymer system being substantially free of a release agent.

25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915

14. The combination according to claim 9 wherein the polymer system for said receiving sheet comprises poly(caprolactone) polyester.

15. The combination according to claim 14 wherein the polymer system for said receiving sheet additionally comprises a second polyester resin comprised of aromatic diacids and an aliphatic diol.

16. The combination according to claim 1 wherein the polymer for said donor sheet is a poly(vinyl butyral) resin.

17. The combination according to claim 16 wherein the polymer system for said receiving sheet comprises polystyrene

18. The combination according to claim 17 wherein the polymer system for said receiving sheet additionally comprises a liquid crystal polymer.

19. A process for thermal diffusion transfer imaging comprising placing a donor sheet and an image-receiving sheet adjacent to one another and heating selected portions of the donor sheet so as to transfer said image-forming material from the donor sheet to the receiving sheet, the donor sheet comprising a support, an image-forming material capable of being transferred by heat and a polymer system comprising at least one polymer as a binder for the image-forming material, and the receiving sheet comprising a polymer system comprising at least one polymer capable of receiving said image-forming material from said donor sheet upon application of heat thereto, the polymer system of said receiving sheet being incompatible/immiscible with the polymer system of said donor sheet at the receiving sheet/donor sheet interface so that there is no adhesion between the donor sheet and the receiving sheet during thermal processing, said donor sheet polymer system and said receiving sheet polymer system being substantially free of a release agent.

20. A process for thermal imaging according to claim 19 wherein said donor sheet polymer system and said receiving sheet polymer system are substantially free of release agents selected from the group consisting of silicone-based oils, poly(organosiloxanes), fluorine-based polymers, fluorine- and phosphate-containing surfactants, fatty acid surfactants and waxes.

21. A process for thermal imaging according to claim 19 wherein said receiving sheet additionally comprises a support material.

22. A process for thermal imaging according to claim 19 wherein said receiving sheet polymer is an extruded polymer film.

23. A process for thermal imaging according to claim 19 wherein said image-forming material is a dye.

24. A process for thermal imaging according to claim 19 wherein the polymer system for said receiving sheet additionally comprises a second polymer forming a polymer blend.

25. A process for thermal imaging according to claim 19 wherein said donor sheet polymer system comprises a blend of two or more polymers as the binder for said image-forming material.

26. A process for thermal imaging according to claim 19 wherein the polymer for said donor sheet is an acrylate resin.

27. A process for thermal imaging according to claim 26 wherein said acrylate resin is poly(methyl methacrylate).

28. A process for thermal imaging according to claim 27 wherein the polymer system for said receiving sheet comprises poly(caprolactone) polyester.

29. A process for thermal imaging according to claim 28 wherein the polymer system of said receiving sheet additionally comprises a second polyester resin comprised of aromatic diacids and an aliphatic diol.

30. A process for thermal imaging according to claim 27 wherein the polymer system for said receiving sheet comprises poly(2,2-dimethyl-1,3-propylene succinate) polyester.

31. A process for thermal imaging according to claim 30 wherein the polymer system for said receiving sheet additionally comprises a second polyester resin comprised of aromatic diacids and an aliphatic diol.

32. A process for thermal imaging according to claim 27 wherein the polymer system for said receiving sheet comprises poly(ethylene adipate) polyester.

33. A process for thermal imaging according to claim 32 wherein the polymer system for said receiving sheet additionally comprises a second polyester resin comprised of aromatic diacids and an aliphatic diol.

34. A process for thermal imaging according to claim 19 wherein the polymer for said donor sheet is a poly(vinyl butyral) resin.

35. A process for thermal imaging according to claim 34 wherein the polymer system for said receiving sheet comprises polystyrene.

36. A process for thermal imaging according to claim 35 wherein the polymer system for said receiving sheet additionally comprises a liquid crystal polymer.

\* \* \* \* \*